

# UNITED STATES PATENT OFFICE.

FREDERICK G. KEYES, OF CAMBRIDGE, MASSACHUSETTS, ASSIGNOR TO COOPER HEWITT ELECTRIC COMPANY, OF HOBOKEN, NEW JERSEY, A CORPORATION OF NEW JERSEY.

## PRODUCTION OF METALLIC TUNGSTEN.

1,293,117.

Specification of Letters Patent.

Patented Feb. 4, 1919.

No Drawing. Original application filed February 11, 1914, Serial No. 818,008. Divided and this application filed July 11, 1917. Serial No. 179,934.

*To all whom it may concern:*

Be it known that I, FREDERICK G. KEYES, a citizen of the United States, and resident of Cambridge, county of Middlesex, State 5 of Massachusetts, have invented certain new and useful Improvements in the Production of Metallic Tungsten, of which the following is a specification.

The present method of obtaining metallic 10 tungsten consists in adding to tungsten tri-oxid ( $WO_3$ ) a suitable binding material, and then reducing in an atmosphere of hydrogen at a high temperature. The ingot thus produced consists of metallic tungsten 15 cemented together by a binding material and the next step in the process is that of subjecting the ingot to a swaging process which is also carried out at a high temperature. The swaging is continued until the 20 ingot is reduced to a diameter that permits of its being drawn while hot through suitable dies until the desired sizes are obtained. The binding material is so selected as to toughen the resulting wire.

25 It is a disadvantage appertaining to this process that the dies are lubricated with graphite. It is a matter of common knowledge that tungsten has a great avidity for carbon, whereas it would be an advantage 30 to prevent, if possible, any cementation. This is done in the above mentioned method of obtaining tungsten and the result is that the tungsten wire used in tungsten lamps is in reality not a pure metal, but a mixture, 35 chemical or otherwise, of binding material and carbid.

Experience shows that a pure metal is very much more ductile than any of its alloys. The object of the present invention is to provide means for obtaining pure metallic 40 tungsten in distinction from tungsten-tungsten carbid.

To accomplish this I dissolve tungsten tri-oxid in boric acid at  $1200^{\circ}$  to  $1400^{\circ}$  C. 45 and electrolyze the solution thus formed. While it is impossible to electrolyze tungsten from an aqueous solution, it is readily possible to secure a deposit of pure metallic

tungsten from a boric acid solution at the temperatures mentioned above. The tungsten can be deposited electrolytically upon a fine tungsten wire and when a sufficient amount has been deposited, it may be subjected to a drawing process such as is now used, or, preferably it may in the early 50 stages of the drawing be drawn through dies of a special tungsten-iron-carbon alloy. Such alloys are already known in the arts and tools made of it hold their edge at a red heat. The pure tungsten having, as 55 stated, a superior quality of ductility when obtained by my process may be drawn through these special dies, thus avoiding the expensive diamond dies. As a lubricating material powdered talcum may be substituted for the deleterious graphite.

This application is a division of my application Serial Number 818,008, filed February 11th, 1914.

I claim as my invention:

1. The method of obtaining pure metallic tungsten which consists in forming a solution of tungsten in boric acid and electrolyzing the solution thus formed.

2. The method of obtaining pure metallic 75 tungsten which consists in dissolving tungsten in boric acid at approximately  $1200^{\circ}$  to  $1400^{\circ}$  C. and electrolyzing the solution thus formed.

3. The method of obtaining tungsten, 80 which consists in forming a solution of tungsten compound in an ionizing medium and electrolyzing the solution thus formed.

4. The method of obtaining tungsten, 85 which consists in dissolving tungsten compound in an ionizing medium at approximately  $1200^{\circ}$  to  $1400^{\circ}$  centigrade and electrolyzing the solution thus formed.

Signed at Cambridge, in the county of Middlesex and State of Massachusetts, this 90 9th day of July, A. D. 1917.

FREDERICK G. KEYES.

Witnesses:

WALTER HUMPHREYS,  
WILLIAM JACKSON.